

No. 856,251.

PATENTED JUNE 11, 1907.

C. HAGSTROM.  
MOLD FOR MAKING STEEL CASTINGS.  
APPLICATION FILED AUG. 28, 1906.

Fig. 1.



Fig. 2.



Witnesses;

P. X. Pezzetti  
E. Batcheller

Inventor;

C. Hagstrom

by - Right Hon. James May  
Attorneys.

# UNITED STATES PATENT OFFICE.

CARL HAGSTROM, OF LYNN, MASSACHUSETTS.

## MOLD FOR MAKING STEEL CASTINGS.

No. 856,251.

Specification of Letters Patent.

Patented June 11, 1907.

Application filed August 28, 1906. Serial No. 332,381.

*To all whom it may concern:*

Be it known that I, CARL HAGSTROM, of Lynn, in the county of Essex and State of Massachusetts, have invented certain new and useful Improvements in Molds for Making Steel Castings, of which the following is a specification.

My invention relates to the making of castings, being especially applicable to the production of large steel castings in sand or similar molds of finely divided refractory material.

Ordinarily in metal founding, the contact surface for the molten metal is produced upon the interior of the matrix by tamping the sand in the flask firmly about a pattern, which is then withdrawn. It is found, however, that the intense heat of the metal introduced burns or so acts upon the surface of the sand that portions become detached, and are embedded in the casting, making it difficult to machine.

The principal object of my invention is to produce a casting free from this defect, thus greatly increasing the ease and economy of working.

Of the accompanying drawings forming a part of this specification,—Figure 1 shows in vertical section the upper or cope portion of a mold arranged in accordance with my invention. Fig. 2 shows a top plan view of the same.

This invention may be carried out by various forms of molds, and by protecting their surfaces wholly or partially, but it is particularly useful in connection with large castings having angular or other portions from which the sand is especially liable to become displaced, or what may be called "danger points." The general application of the invention being understood, it will be here described by reference to one embodiment in which only these danger points are to be protected.

In the drawings, 10 designates the cope of an ordinary two-part flask, in which the sand matrix 11 has been tamped about a pattern to produce its half of the depression furnishing the mold, a passage or gate 12 being formed through the sand for the introduction of the molten metal. The mold is shown as having a corner or angular portion 13 at the meeting of two surfaces, and this might be loosened by the metal when poured, as has been previously described. To prevent this and to secure a simple and perfect casting, I

place over this portion of the mold surface, causing it to substantially conform thereto, a lining 14 of some material which will be melted by the heat of the substance to be cast. This lining is preferably of very thin sheet metal, say  $1/64''$  in thickness, and of any suitable surface dimensions, and being of the same character as that forming the casting. The lining sheets may be secured in place by nails 15, driven through the corners or wherever is necessary into the densely packed sand. As the metal flows through the gate, the sand is protected by the lining, so that the surface sand is not burned and separated from the remainder of the matrix. As soon as the molten metal fairly comes into contact with the lining, the latter liquefies and becomes a portion of the casting, bringing the metal against the surface of the sand, but as the former is now somewhat chilled, all danger of loosening the sand is passed. Thus it will be seen that the casting will be true to all the mold surfaces, yet be entirely free from sand.

I claim:

1. A mold for casting, which comprises a sand matrix, and a lining consisting of a solid which will be liquefied by the heat of the substance cast.

2. A mold for metal founding, comprising a matrix of finely divided refractory material, and a lining consisting of a metal which will be liquefied by the heat of the metal cast.

3. A mold for metal founding, comprising a matrix of finely divided refractory material, a lining consisting of sheet metal generally conforming to the surface of the matrix, and means for securing the lining to the matrix, said lining being composed of a metal which will be liquefied by the heat of the metal cast.

4. A mold for metal founding, comprising a matrix of sand, a lining of sheet metal generally conforming to the surface of the matrix, and securing means passing through the sheet metal into the sand, said lining being composed of a metal which will be liquefied by the heat of the metal cast.

In testimony whereof I have affixed my signature, in presence of two witnesses.

CARL HAGSTROM.

Witnesses:

H. BROWN,  
E. BATCHELDER.